

Nov. 30, 1926.

1,608,709

R. VAN A. MILLS

METHOD OF AND MEANS FOR PREVENTING CORROSION OF WELL TUBING,  
CASING, AND WORKING BARRELS

Filed Sept. 10, 1924

2 Sheets-Sheet 2



Fig. 10.



Fig. 11.



Fig. 12.



Fig. 8.



Fig. 9.



Fig. 13.

Inventor

Ronald Van Auklen Mills.

By Munson H. Lane.

Attorney

Nov. 30, 1926.

1,608,709

R. VAN A. MILLS

METHOD OF AND MEANS FOR PREVENTING CORROSION OF WELL TUBING,  
CASING, AND WORKING BARRELS.

Filed Sept. 10, 1924 2 Sheets-Sheet 1



Inventor  
Ronald Van Auken Mills.

884

Munson H. Lane

Attorney

## UNITED STATES PATENT OFFICE.

RONALD VAN AUKEN MILLS, OF SANDY SPRING, MARYLAND, ASSIGNOR TO PETER Q. NYCE, OF WASHINGTON, DISTRICT OF COLUMBIA.

METHOD OF AND MEANS FOR PREVENTING CORROSION OF WELL TUBING, CASING, AND WORKING BARRELS.

Application filed September 10, 1924. Serial No. 737,010.

The invention relates to a method of and means for protecting well tubing, casing, working barrels, and the like, from corrosion. The invention is particularly designed for use in oil wells where the loss due to corrosion is very great on account of the highly corrosive action of the saline liquids which are generally found in such wells.

Corrosion of tubing, casing and other equipment in oil and gas wells is essentially an electro-chemical process dependent upon galvanic action where the metallic equipment is wet by water.

Galvanic action between tubing and casing is most serious where the tubing swings close to or against the casing.

The corrosion occurs on electro-positive surfaces, that is to say, the surfaces from which an electric current leaves a metal and passes into an electrolyte like salt water.

To stop this corrosion in oil and gas wells it is desirable to:

1. Space the tubing from the casing.
2. Render the equipment electro-negative.
- 25 3. Supply an electropositive material that will corrode in preference to the iron or other metal in the equipment.

It is the purpose of this invention to accomplish these things.

30 The invention will be described under three headings, covering different phases of the invention, although all the features herein described cooperate to produce a unitary result, namely the prevention of corrosion.

35 The features which will now be discussed in detail are (1) the insulating tubing spacers, (2) the electropositive metal sleeve, and (3) the metallic contact brush.

40 *Tubing spacers.*

To prevent the serious corrosion that results from tubing swinging close to or against the casing, the present invention consists first of a non-conducting tubing spacer fitting on the tubing and held in place by the tubing collar or other projections on which it rests. The spacers may also be held in place by friction, clamps, screws or any other suitable device. The spacers are made 45 of bakelite fiber or some like non-conducting material. They are circular disks perforated by holes to allow the passage of fluids and having a hole in the center just large enough for the snug passage of the tubing. Other sleeves.

55 shapes of non-conducting spacers may be used in the spirit and embodiment of this first part of the invention which consists essentially of a non-conducting tubing spacer.

The tubing spacers may be used with or without the other parts of the device here- 60 inafter described.

*Electropositive metal sleeve.*

Since corrosion occurs on an electro-positive surface, the second part of this invention consists of a sleeve of metal such as 65 zinc that is electropositive to iron and therefore when properly placed in the galvanic system in the well is positive to the iron and renders the iron electro-negative. The zinc, 70 being the electropositive metal, is corroded whereas the iron is protected at the expense of the zinc. The zinc must be replaced from time to time, at intervals of from six months to a year, as it is consumed. 75

By placing the zinc on the tubing and using spacers to prevent the zinc and the tubing from coming in contact with the casing, except where desired as for instance above the water level inside the well, it is 80 possible to make the tubing with its superimposed zinc the positive electrode in the galvanic system of which the casing is the negative electrode. Moreover, the zinc on the tubing being electropositive with respect 85 to the tubing, protects the tubing as well as the casing.

Contact between the tubing and casing is made above the water level either through the casing head or through actual contact between tubing and casing in the well where the tubing swings against the casing, or through a special device hereinafter described.

For the working of this method of protection it is imperative to have the best possible electrical contact between zinc and tubing and the best possible electrical conductivity in the tubing and casing throughout the galvanic circuit. It is also imperative 100 to prevent short circuiting between the zinc and the casing and between the tubing and casing below the water level, for such short circuiting will consume zinc unnecessarily or cause corrosion or both. This is accomplished through the use of the tubing spacers alone, and in conjunction with the zinc sleeves. The combined use of the spacers 105

with a zinc sleeve constitutes the second part of this invention, a device for the protection of well tubing and casing against corrosion.

*Metallic contact brush.*

The third part of the invention consists of a metallic contact brush attached to the tubing above the water level, its purpose being to complete the galvanic circuit above the water level and to avoid the unnecessarily long circuit around through the casing head.

The use of the contact brush is not essential though it should increase the efficiency of the zinc protection.

The invention will be more clearly understood by reference to the accompanying drawings, in which:

Fig. 1 is a view partly in section and partly in elevation showing one form of the protective sleeve applied to well tubing, the sleeve being equipped with insulating spacers.

Fig. 2 is a plan view of the construction shown in Fig. 1, looking down upon the spacer.

Figs. 3 and 4 are details in elevation and plan, respectively, showing the tubing spacers.

Fig. 5 is a detail view showing a spring washer to be applied at the top of the protective sleeve, and serving to maintain electrical contact between the sleeve and the tubing.

Fig. 6 is a view similar to Fig. 1 showing a modified form of the electropositive metal sleeve.

Fig. 7 is a detail view showing a modified form of tie rod for securing together the protective sleeve and spacing elements.

Fig. 8 is an elevation showing another modification of the protective sleeve wherein the sleeve is spaced away from the tubing, but not from the casing.

Fig. 9 represents a further modification of the zinc sleeve wherein a space is provided between the sleeve and the tubing adapted to receive molten metal or other material making a cast or welded connection between the zinc and the tubing.

Fig. 10 is a diagrammatic view showing the galvanic circuit which exists in a well employing the electropositive metal sleeve in connection with the well tubing.

Fig. 11 is a similar view showing the circuit where a special metallic contact brush is employed.

Fig. 12 is a detail view showing one form of contact brush, and

Fig. 13 is a view similar to Fig. 12, but showing a different form of contact brush.

According to the present invention, sleeves of zinc (or other metal which is electropositive with respect to iron), are fitted over the tubing so as to be in contact with the

tubing but spaced away from the casing so as to prevent direct contact therewith. The term "electropositive metal" as herein used signifies a metal from which an electric current passes through an electrolyte to iron or some other metal with which the electropositive metal forms a galvanic couple. Insulating spacers at the ends of the zinc sleeve and extending beyond the zinc sleeve are provided to protect the zinc against impact and abrasion and to prevent the zinc from swinging against the casing.

By spacing the zinc away from the casing, short circuiting between the zinc and the casing, and the consequently excessive consumption of the zinc are prevented.

The zinc sleeve being electropositive with respect to both the tubing to which it is attached and the casing with which it is in close proximity, serves to prevent corrosion of both the tubing and the casing, the zinc itself being attacked by the corrosion in preference to the iron or steel.

The arrangement described above may be reversed, so that the zinc sleeve though attached to the tubing is in contact with the casing but not with the tubing.

It will be further understood that any desired number of the protecting sleeves may be employed without departing from the spirit of the present invention.

Referring particularly to Figs. 1 and 2, the reference numeral 10 indicates the tubing in a well (oil well or any other kind of well) which is normally subjected to the corrosive action of liquids and gases, the usual tubing collar being indicated at 11. The well casing is indicated by the numeral 12.

In order to prevent corrosion of the tubing and casing, a sleeve 13 composed principally of zinc or other metal which is electropositive with respect to iron, is fitted over the tubing and rests upon the spacer 14. The internal diameter of the sleeve is sufficient to allow the tubing to pass through freely so that the sleeve may be easily slipped on to the tubing.

The block of zinc 13 is preferably protected at both ends by means of circular spacers 14 of bakelite, fiber or other like insulating material which prevents the zinc from swinging against the casing, the diameters of the spacers being greater than the diameter of the zinc sleeve. The spacers 14 may be held in place merely by gravity or may be secured to the zinc sleeve in any suitable manner, as by means of tie bolts 15. The bottom spacer rests by gravity on top of the tubing collar, the zinc resting on top of the spacer.

In many instances it may be found desirable to provide shoulders 20 upon the tie rods 15 in order to hold the spacers 14 in spaced relation even after the zinc sleeves

13 have disintegrated due to corrosive action. This arrangement is shown in Fig. 7.

Preferably, also, a spring sleeve 16 is provided at the top of the zinc sleeve 13, having projections 17 extending a short distance into the space between the zinc and the tubing, whereby a good electrical contact is secured and looseness of the zinc sleeve is prevented.

10 While the invention has been described in detail, for the purpose of illustration, it is obvious that many modifications may be employed without departing from the spirit of the invention.

15 For example, in Fig. 6, is shown an arrangement consisting merely of a plurality of zinc castings 18 surrounding the tubing 10, spacing members 14 being provided between the zinc castings as shown.

20 Where the device is used in connection with oil wells, it is desirable to provide means to permit the free passage of gas or other fluids between tubing and casing. Accordingly, the spacers 14 are provided with 25 a plurality of holes 19 for the passage of fluids.

Another modification of the device which falls within the scope of the invention is shown in Fig. 8. According to this arrangement, the zinc sleeve 13 is completely insulated from the tubing by means of a sleeve 21 of bakelite fiber or other insulating material which may be formed integral with the bakelite spacer 14. According to this arrangement, the zinc sleeve may be of greater diameter than the spacer 14, and is preferably of such size as to fit loosely within the outer casing 12. With this arrangement, the insulation is located between the tubing and zinc sleeve, rather than between the casing and the sleeve as in the previous embodiments of the invention.

40 Fig. 9 represents a further modification of the zinc sleeve wherein a space 22 is provided between the sleeve 13 and the tubing 10 adapted to receive molten metal or other material making a cast or welded connection between the zinc and the tubing. The purpose of casting or welding the sleeve is to give the best possible contact between the zinc and the tubing.

45 Referring now to the diagrammatic representation of the galvanic circuit shown in Fig. 10, it will be seen that the current flows in the direction of the arrows from the electropositive metal 13 through the electrolyte 23 (saline water or other corrosive liquid) to the casing 12. The circuit is completed through the casing head 24 and the tubing 10.

If desired, metallic contact brushes 25 as shown in Fig. 11, may be used to complete the galvanic circuit above the water level so as to avoid the unnecessary long circuit through the casing head.

One form of contact brush is shown in detail in Fig. 12. According to this embodiment of the invention resilient metal wires 30 are inserted through holes 31 in a metal sleeve 32 surrounding the well tubing 10. These wires are bent to U-shape and make a good electrical contact between the tubing 10 and casing 12.

A simpler form of contact brush is shown in Fig. 13 in which wires 33 are merely twisted about the tubing 10, and if desired, may be spot welded thereto as at 34, or fastened together to make a wire sleeve fitting around the tubing.

The invention has been described in great detail for the purpose of illustration, but it is evident that it is subject to many modifications within the scope of the appended claims.

I claim:—

1. A method of preventing corrosion of well tubing and casing which consists in providing non-conducting spacing rings between said tubing and casing, whereby said tubing is prevented from swinging close to or against said casing.

2. Means for preventing corrosion of well tubing and casing comprising a plurality of non-conducting spacing rings secured at intervals upon said tubing to prevent the tubing from swinging against said casing, said spacers being perforated to permit passage of fluid.

3. In combination with well tubing and casing, a plurality of non-conducting spacing rings interposed between said tubing and the casing, said ring being provided with a plurality of apertures to permit the passage of fluid.

4. The method of protecting tubing against corrosion which consists in providing said tubing with a sleeve of metal electro-positive with respect to iron, and supplying insulating spacers above and below said metal sleeve.

5. The method of protecting well tubing or casing against corrosion which consists in providing a metal sleeve composed of material which is electro-positive with respect to the tubing or casing in close proximity to said tubing or casing, but spaced therefrom.

6. The method of protecting tubing or casing composed of ferrous material which consists in providing a zinc sleeve in close proximity to said tubing or casing but spaced therefrom.

7. The method of protecting well tubing against corrosion which consists in providing said tubing with a sleeve of metal which is electro-positive with respect to the tubing and providing a non-conducting spacer below said metal sleeve.

8. A method of protecting well tubing and casing against corrosion which consists in

- interposing between said tubing and casing a plurality of sleeves composed of metal which is electro-positive with respect to the tubing and casing, preventing short circuiting between said tubing and casing at said electro-positive sleeves by the use of suitable insulators, and electrically connecting said tubing and casing above the liquid level in the well.
- 10 9. In combination with well tubing and casing, a protective metal sleeve upon said tubing and an insulating sleeve between said protective sleeve and said tubing.
- 10 10. A device for protecting well tubing and casing against corrosion comprising, in combination, a plurality of zinc sleeves surrounding the tubing and in contact therewith located below the level of the liquid in the well, non-conducting spacing rings of greater diameter than the zinc for preventing contact between said sleeve and said casing, and contact devices above the level of the liquid in the well for completing an electric circuit.
- 25 11. The method of protecting tubing against corrosion which consists in supply- ing a sleeve of metal which is electropositive to the tubing, in close proximity to the tubing, but spaced therefrom.
12. In combination with a well tubing and casing, a plurality of zinc castings surrounding said tubing at intervals, and bakelite, fiber or other spacing members of greater diameter than the zinc castings interposed between the castings and designed to prevent said castings from swinging against said casing.
13. In combination with a well tubing and casing, a zinc sleeve surrounding the tubing in close proximity thereto, but not in direct contact therewith, an insulating sleeve interposed between zinc and the tubing, a collar on said tubing, and an insulating spacer integral with said insulating sleeve, and resting upon said collar, said insulating sleeve being of less diameter than the zinc sleeve, and said zinc sleeve fitting closely within the outer casing.

In testimony whereof I affix my signature.

RONALD VAN AUKEN MILLS.